

F. SIGNORET,  
FUMIGATING COMPOSITION,  
APPLICATION FILED FEB. 10, 1914.

1,159,109.

Patented Nov. 2, 1915.

Fig. 1.



Fig. 2.



WITNESSES:

John C. Sanders  
Albert F. Hauman

INVENTOR:

by Ferdinand Signoret  
Mr Wallace White

ATTY

# UNITED STATES PATENT OFFICE.

FERDINAND SIGNORET, OF MARSEILLE, FRANCE.

## FUMIGATING COMPOSITION.

1,159,109.

Specification of Letters Patent.

Patented Nov. 2, 1915.

Application filed February 10, 1914. Serial No. 817,751.

To all whom it may concern:

Be it known that I, FERDINAND SIGNORET, a citizen of France, residing at 8 Place de la Bourse, Marseille, in the Republic of France, have invented new and useful Improvements in Fumigating Compositions, of which the following is a specification.

Sulfurous acid is the gas mainly employed for fumigating or sterilizing casks, wine 10 vats, etc. It is also largely used for other disinfecting purposes. In order to produce this gas, sulfur "wicks" may be burnt, composed of canvas, paper or other substance forming a skeleton which is then coated 15 with sulfur. These wicks of various forms have the disadvantage of allowing drops of fused sulfur to drop into the casks or vats, &c. Various disadvantages result from this: For instance, the sulfur spread on the strips 20 of canvas, paper or other substance, loses a considerable percentage of its bulk by melting and running, and this molten sulfur is extinguished in contact with the damp part of the cask or with the liquid, in the case 25 of a vat which is being emptied. Hence it is impossible to use the entire mass and when the ignited drop meets the liquid or the damp wood, sulfureted hydrogen may be formed which then communicates to the 30 whole receptacle its characteristic and nauseating odor.

The object of the present invention is an improved composition which avoids all these disadvantages, and has the property of 35 burning in its entirety, without fused sulfur running. This result is obtained by manufacturing it in the following way:— Sulfur in grains or in coarse powder is mixed with ordinary silicate of soda and 40 this mixture is dried after it has been molded or pressed into slabs which have been divided into tablets. In order to make these tablets grind 100 kilograms of sulfur in order to conform it into grains of about 3 45 millimeters. Pour the coarse powder thus obtained into 35 liters of silicated soda or of commercial potash, which mixture is then stirred in order to obtain an intimate mixture in the form of paste. This paste is 50 transformed under a roller into the form of slabs 8 millimeters thick, which are passed under polishing rollers coated with flowers of sulfur to powder the same and thus prevent adhesion. The slabs are passed after- 55 ward under a winged roller that divides the

slab into tablets by tracing the longitudinal division, the transverse division and the grooves and perforations in the respective tablets being formed by passing the slabs through another machine for this purpose. 60 These grooves permit the subsequent breaking of the slabs into separate tablets. One may, if desired, obtain the tablets by means of a simple press. The tablets thus obtained are then dried in any convenient manner and 65 will be rendered thereby very homogeneous and rigid. Each tablet will weigh about 100 grams and is divided into a number of parts.

In the accompanying drawings:—Figure 70 1 is a plan view of a slab of brimstone after it has been molded; Fig. 2 is a section on the line 1—1 of Fig. 1.

This tablet is divided into twenty parts A by means of grooves C and then each of 75 these parts is again divided into two by grooves D. Each of these parts is perforated with a hole B, to enable it to be suspended in the cask by a wire, an incombustible cord, or any other means. The residue from the combustion is a mass somewhat resembling pumice stone, which remains attached to its means of suspension.

It is quite evident that the product may be made in the form of tablets, as hereinbefore indicated, or in the form of cubes, rods, cylinders, lozenges, and the like. The same result may also be obtained by immersing a cellular substance, such as felt in fused sulfur. 90

I claim:

1. The herein described process for the manufacture of a fumigating product consisting in mixing comminuted sulfur in the form of grains of approximately 3 millimeters in diameter with a solution of soluble silicate of an alkali metal to coat the grains, in drying this mixture, and then in molding the substance to a convenient form. 95

2. A fumigating product in the form of 100 an intimate mixture of sulfur in the form of grains of substantially 3 millimeters in diameter, and silicate of an alkali metal.

In testimony whereof I have signed my name to this specification in the presence of 105 two subscribing witnesses.

FERDINAND SIGNORET.

Witnesses:

EUGENE DUCASSOU,  
PAUL H. CRAM.